

Dec. 24, 1940.

G. V. HALLMAN

2,225,778

CAN BODY BLANK PREPARING METHOD

Filed March 6, 1939



INVENTOR  
G. V. Hallman  
Mason, Porter  
ATTORNEYS

## UNITED STATES PATENT OFFICE

2,225,778

## CAN BODY BLANK PREPARING METHOD

George V. Hallman, River Forest, Ill., assignor to  
Continental Can Company, Inc., New York,  
N. Y., a corporation of New York

Application March 6, 1939, Serial No. 260,196

2 Claims. (Cl. 91—70.3)

The invention relates generally to the art of can making and primarily seeks to provide a novel method of preparing can body blanks of black plate or mild steel, or principally the edge portions of the blanks which are to form the can body seams, so as to facilitate subsequent solder bonding of the can body seams.

Untreated black plate oxidizes when exposed to the air, and scale forms thereon which interferes with the solder adhering to the plate when it is attempted to solder side seams of cans formed from such plate. The present invention seeks to remedy this condition and make possible economical formation of cans from relatively inexpensive black plate by providing a novel method in which the edge portions only of the black plate which are to be formed into side seams in the making of the cans are first cleaned of oxidation and scale and then given a suitable metallic coating, preferably tin, so as to facilitate subsequent soldering.

In its more detailed nature, the invention resides in the steps of pickle bath or otherwise cleaning the edge portions of the black plate blanks which are to be formed into side seams, and then bending the blanks and immersing the cleaned edge portions thereof in a coating bath to suitably plate said edge portions so as to facilitate subsequent soldering thereof.

Another object of the invention is to provide a method of the character stated in which the pickling and tin plating steps are performed successively on continuously moving black plate can body blanks.

Another object of the invention is to include in the method the steps of treating the plated edge portions to determine the thickness of the plating thereon, and of buffing said plated edges.

With the above and other objects in view that will hereinafter appear, the nature of the invention will be more fully understood by following the detailed description, the appended claims, and the several views illustrated in the accompanying drawing:

In the drawing:

Figure 1 is a diagrammatic longitudinal section illustrating the invention.

Figures 2 and 3 are vertical cross sections taken on the lines 2—2 and 3—3 on Figure 1.

Figures 4 and 5 are vertical cross sections respectively illustrating the abrading and buffing steps.

Figure 6 is a perspective view of a can body blank prepared in accordance with the invention.

In the drawing I have diagrammatically illus-

trated one manner of practicing the invention in which body blanks 5 to be formed into can bodies are moved by a conveyor 6 through a stationary horn or horse structure 7 so shaped as to receive the body blanks in flat horizontal condition and gradually turn the lateral edge portions thereof downwardly in inverted U-shape as illustrated in Figure 2. The horn or horse structure diagrammatically illustrated in Figures 1, 2 and 3 is formed to include successively effective edge turning portions, with a restoring or edge straightening portion following each edge turning portion, so that when passing through this structure each can body blank 5, horizontally received, will have its lateral edge portions turned downwardly in inverted U-shape, then upwardly to restore the blank to its flat horizontal position, then downwardly to again form the blank into inverted U-shape, and then again upwardly to restore the blank to its horizontal flat condition.

Thus the blank is twice formed into inverted U-shape and twice restored to its flat horizontal condition. During the first bending of the lateral edge portions of the blank, said edge portions are immersed in a suitable pickling bath 8 after which the blank is restored to its flat condition so that it can pass away from the pickling bath. The edge portions of the blanks are turned downwardly for the second time over a tinning bath 9 of molten tin. This bath is covered by a thin depth of flux indicated at 10. By reason of the provision of the successive pickling and tinning baths 8 and 9, the extreme lateral edge portions only of the blanks 5 will be first pickled and cleaned of oxidation and scale and then receive a tin plating by immersion in the flux covered tinning bath.

By practicing this method of handling the body blanks, the tin plating is provided only at the edge portions of the blanks which are to be subsequently formed into side seam structures. Thus efficient solder bonding of the side seams is assured with the use of a minimum amount of tin.

After the body blanks leave the tinning bath they are edge treated so as to determine the thickness of the tin plating and to buff or polish this plating. In the diagrammatic illustration herein made, the blanks are illustrated as passing through suitable feed rollers 11 and successively positioned abrading rolls 12 and buffing rolls 13. See Figures 1, 4 and 5. The abrading rolls 12 may be adjustably mounted so as to reduce to the thickness desired the tin plating acquired by immersion in the bath 9, and the buffing rolls 13

serve to suitably polish the plating reduced to the desired thickness.

In Figure 6 of the drawing a body blank 5 formed of black plate or mild steel is illustrated with an edge plating of tin applied to the lateral edge portions at the respective faces thereof as illustrated at 14.

While I have referred herein specifically to immersing the edge portions of the can body blanks in a tin plating bath, the invention is not to be considered limited to plating with tin. The edge portions of the blanks may be immersed in any metallic plating bath suitable for use on black plate to facilitate soldering operations. For example, plating baths of lead, zinc or copper may be used as well as the tin specifically mentioned hereinabove.

It is to be understood that the method can be practiced by use of any suitable mechanism including means capable of suitably bending the blanks so that the edge portions only thereof will be immersed in the pickling and plating baths. This bending of the blanks may take place while they are continuously traveling, or the bending may be formed during rest intervals of the blanks.

I claim:

1. The method of preparing black plate can body blanks for formation into can bodies in which the side seams are soldered which com-

prises, continuously conveying the individual blanks in spaced and aligned relation with the edge portions thereof subsequently to be formed into can body side seams disposed laterally and in the direction in which the blanks are being 5 conveyed, successively passing said blanks over a pickling bath and a metallic plating bath, and bending the blanks so as to depress the lateral edge portions only thereof for immersion in said baths to the extent to which said edges are to 10 be used in the formation of can body side seams.

2. The method of preparing black plate can body blanks for formation into can bodies in which the side seams are soldered which comprises, continuously conveying the individual 15 blanks in spaced and aligned relation with the edge portions thereof subsequently to be formed into can body side seams disposed laterally and in the direction in which the blanks are being 20 conveyed, successively passing said blanks over a pickling bath and a metallic plating bath, bending the blanks so as to depress the lateral edge portions only thereof for immersion in said 25 baths to the extent to which said edges are to be used in the formation of can body side seams, abrading the plated edges to determine the thickness of the plating, and buffing said plated edges.

GEORGE V. HALLMAN.